

## UNITED STATES PATENT OFFICE.

JOSEPH BLACK, OF LOS ANGELES, CALIFORNIA.

## PROCESS OF MANUFACTURING LIQUID FUEL.

No Drawing.

Application filed September 27, 1923. Serial No. 665,183.

*To all whom it may concern:*

Be it known that I, JOSEPH BLACK, a citizen of the United States, residing at Los Angeles, in the county of Los Angeles and 5 State of California, have invented certain new and useful Improvements in Processes of Manufacturing Liquid Fuel, of which the following is a specification.

This invention relates to a process of manufacturing liquid fuel and the products derived therefrom, and has for its general object to provide, in a manner as herein-after set forth, a liquid fuel for use in internal combustion engines or for any purposes for which the fuel is found applicable, which while capable of production at a cost below that of the well known gasoline of commerce, will be more efficient than 10 the latter in the matter of power development, mileage per gallon, reducing carbonization to an absolute minimum to assure constant free running of an engine, and ease in starting power in cold weather, and the 15 foregoing several advantages are accomplished by the use of a liquid fuel manufactured in accordance with the process forming the subject matter of my invention.

In the production of a liquid fuel, in accordance with this invention, I employ a base of crude petroleum and raw coal oil, or what is known to the trade as untreated coal oil. The crude petroleum and raw coal oil in the desired quantities are mixed together in a suitable still and to such mixture is added in the desired proportions, acetone, benzole, salsoda and wood or denatured alcohol. The composition as stated is then 30 subjected to the action of compressed cold air to provide for a thorough agitation to obtain the complete admixing of the several constituents of the composition. After the agitation, the composition is submitted to 35 heat and brought to a temperature of one hundred twenty degrees Fahr., and after the composition has reached the temperature referred to, it is subjected to the action of dry steam to what may be termed preserve the acetone, benzole, salsoda and alcohol so they will perform their function in 40 the ultimate product, or in other words dry steam is applied to prevent the burning up of the acetone, benzole, salsoda and alcohol.

The supply of dry steam is continued until the process has been completed. 55

Immediately after the beginning of the subjecting of the composition to dry steam, the composition starts to run or come over through a condenser into a storage tank. 60 The come-over or run starts at about seventy-five or eighty proof gravity and is discharged from the still as a watery white liquid into the tank and when the supply to the tank has been shut off, the fuel therein will be of fifty-eight proof gravity. The supply to the tank is continued until the 65 temperature of the composition in the still has reached four hundred twenty degrees Fahr., and by this time the come-over or run discharged into the tank will reach one hundred gallons and an end point of 437, as is required. When the composition in the 70 still is at four hundred twenty degrees Fahr., the come-over or run is then shut off to the tank and conducted to a secondary tank, and the supply to the latter will amount to seventy-three gallons of forty-five proof gravity with an end point of 480. 75 The composition within the still, as the come-over or run is supplied to the secondary tank, reaches four hundred eighty degrees Fahr., and will stand as such. After the secondary tank has been shut off to the 80 still, the residuum of the composition remaining, amounting to approximately twenty-five gallons of thirty-two proof gravity, is removed and utilized for stove oil. 85

The liquid fuel contained in the secondary tank, has combined therewith, in suitable proportions, acetone, benzole, alcohol and casing head gas, and the mixture is thoroughly agitated for a predetermined period, and which will raise the gravity of the fuel to sixty proof, making it an unusually satisfactory fuel having an end point between 470 and 480. 90

As an example of the proportions of the several constituents from which a liquid fuel, in accordance with this invention, is manufactured, I employ one hundred gallons of crude petroleum, one hundred gallons of raw coal oil, or what is known to the trade as untreated coal oil, two gallons of acetone, two gallons of benzole, ten pounds of salsoda and one-half gallon of

wood or denatured alcohol. The proportions, by way of example, of acetone, benzole and alcohol which are admixed with the fuel in the secondary tank, are as follows:—

5 6 14 ounces acetone, 14 ounces benzole, 12 ounces alcohol.

The several constituents added to the petroleum and coal oil act to prevent carbonization, to lower the ignition point or 10 flashing point, providing for the thorough combining of the crude petroleum and coal oil, or rather to form a homogeneous and permanent mixture, as well as acting as a carrying or mixing medium to provide a 15 permanent and homogeneous mixture.

The acetone employed in the fuel in the secondary tank acts as a binder between the coal oil and casing head gas, or in other words, prevents the separation of coal oil 20 from the casing head gas.

What I claim is:—

1. A process of manufacturing a liquid fuel comprising the distilling of a composition consisting of crude petroleum untreated 25 and coal oil in approximately equal volumes combined with a mixture consisting of acetone in the approximate proportion of one-fiftieth of the volume of petroleum, benzole in the approximate proportion of one-fiftieth of the volume of the petroleum, salsoda in the approximate proportion of one-eighthieth of the volume of the petroleum, and alcohol in the approximate proportion of one two-hundredth of the volume of the petroleum to a temperature of one hundred twenty degrees Fahr. to start a come-over or run, then collecting in a receiver the come-over or run until the temperature of the composition reaches four hundred twenty degrees Fahr., thereby providing a liquid fuel of fifty-eight proof 30 gravity and 437 end point, then collecting in an independent receiver the come-over or run until the composition reaches a temperature of four hundred eighty degrees, thereby providing a liquid fuel of forty-five proof gravity and end point of 480, and then raising to sixty proof gravity the liquid fuel of 35 forty-five proof gravity by combining therewith casing head gas, acetone, benzole and alcohol.

3. A liquid fuel obtained by dry steam distillation of approximately equal volumes of each of crude petroleum and raw coal oil distilling over between approximately 120 degrees Fahr., and 420 degrees Fahr., and containing approximately 5% of a mixture of approximately equal parts of each 40 of acetone and benzole and a smaller proportion of alcohol, and water obtained from the dry steam.

4. A liquid fuel obtained by dry steam distillation of approximately equal volumes of each of crude petroleum and raw coal oil distilling over between 420 degrees Fahr., and 480 degrees Fahr., and water obtained from the dry steam.

5. A liquid fuel obtained by dry steam distillation of approximately equal volumes of each of crude petroleum and raw coal oil distilling over between 420 degrees Fahr., and 480 degrees Fahr., and water obtained from the dry steam, combined with casing head gas and a mixture of approximately equal parts of alcohol, acetone and benzole, and water obtained from the dry steam.

tone in the approximate proportion of one-fiftieth of the volume of petroleum, benzole 55

in the approximate proportion of one-fiftieth of the volume of the petroleum, salsoda in the approximate proportion of one-eighthieth of the volume of the petroleum,

and alcohol in the approximate proportion of one two-hundredth of the volume of the petroleum to a temperature of

one hundred twenty degrees Fahr. to start a come-over or run, then collecting in a receiver the come-over or run until the temperature of the composition reaches four hundred twenty degrees Fahr., thereby providing a liquid fuel of fifty-eight proof

gravity and 437 end point, then collecting in an independent receiver the come-over or 60 run until the composition reaches a temperature of four hundred eighty degrees, thereby providing a liquid fuel of forty-five proof

gravity and end point of 480, and then raising to sixty proof gravity the liquid fuel of 65 forty-five proof gravity by combining therewith casing head gas, acetone, benzole and alcohol.

3. A liquid fuel obtained by dry steam distillation of approximately equal volumes 70 of each of crude petroleum and raw coal oil distilling over between approximately 120 degrees Fahr., and 420 degrees Fahr., and containing approximately 5% of a mixture of approximately equal parts of each 75 of acetone and benzole and a smaller proportion of alcohol, and water obtained from the dry steam.

4. A liquid fuel obtained by dry steam distillation of approximately equal volumes 80 of each of crude petroleum and raw coal oil distilling over between 420 degrees Fahr., and 480 degrees Fahr., and water obtained from the dry steam.

5. A liquid fuel obtained by dry steam distillation of approximately equal volumes 85 of each of crude petroleum and raw coal oil distilling over between 420 degrees Fahr., and 480 degrees Fahr., and water obtained from the dry steam, combined with casing head gas and a mixture of approximately

equal parts of alcohol, acetone and benzole, and water obtained from the dry steam.

In testimony whereof, I affix my signature hereto.

JOSEPH BLACK.